

# United States Patent [19]

Thérond

[11] Patent Number: 5,009,734

[45] Date of Patent: Apr. 23, 1991

[54] METHOD OF MAKING AN INSULATING SUPPORT ARM FOR AN ELECTRIC LINE POLE

[75] Inventor: Michel Thérond, Cahors, France

[73] Assignee: Manufacture d'Appareillage Electrique de Cahors, France

[21] Appl. No.: 373,162

[22] Filed: Jun. 29, 1989

## Related U.S. Application Data

[62] Division of Ser. No. 168,510, Mar. 15, 1988, Pat. No. 4,867,399.

## Foreign Application Priority Data

Mar. 20, 1987 [FR] France ..... 87 03885

[51] Int. Cl.<sup>5</sup> ..... B27N 3/00

[52] U.S. Cl. ..... 156/184; 156/191; 156/192; 174/45 R; 248/219.3

[58] Field of Search ..... 52/309.1, 309.7, 309.14; 156/62.6, 62.8, 245, 184, 191, 192; 174/45 R; 248/65, 218.4, 219.3; 428/229

## References Cited

### U.S. PATENT DOCUMENTS

3,408,239 10/1968 Wedin ..... 156/62.8  
3,813,837 6/1974 McClain et al. ..... 174/45 R X  
4,141,929 2/1979 Stoops et al. ..... 156/179 X  
4,220,496 9/1980 Carley et al. ..... 156/245 X

4,682,747 7/1987 King, Jr. et al. ..... 174/45 R  
4,853,279 8/1989 Shibata et al. ..... 428/902

## FOREIGN PATENT DOCUMENTS

919534 2/1963 United Kingdom ..... 174/45 R

Primary Examiner—David A. Simmons

Assistant Examiner—James J. Engel, Jr.

Attorney, Agent, or Firm—Kenyon & Kenyon

## ABSTRACT

Insulating equipment (100) includes a flexible arm (1) having at one of its ends a means for attachment to a pole and at the other end means for attaching an electric line substantially perpendicular to the arm (1). The thickness of the arm (1) decreases regularly from the means of attachment to the pole toward the means of attachment to the electric line, while the height of the cross section of the arm is constant. The arm (1) has in the direction of its thickness a series of layers (7a, 7b, 7c, 7d) of continuous mineral fibers extending in the direction of the arm's length and separated by layers (8a, 8b, 8c, 8d) of randomly-oriented short mineral fibers. These layers are bonded by a synthetic resin in which a layer (9a, 9b) of fabric of mineral fibers may be placed on each side of the arm (1) between the first layer of short fibers and the following layer of continuous fibers. To be used for improving longitudinal flexibility and resistance to vertical loads.

4 Claims, 4 Drawing Sheets











FIG. 7



FIG. 9

## METHOD OF MAKING AN INSULATING SUPPORT ARM FOR AN ELECTRIC LINE POLE

This is a division of application Ser. No. 07/168,510 filed Mar. 15, 1988 now U.S. Pat. No. 4,867,399.

This invention relates to insulating equipment for an electric line pole and to a procedure for manufacturing said equipment.

### BACKGROUND OF THE INVENTION

The electric lines used to carry electricity under low, medium, and high tension are supported by poles or pylons by the use of insulating brackets called "equipment."

In its uses to date, this equipment is made up of metallic pieces provided with means for attachment to the post and with means for hanging the electrical lines in a direction perpendicular to the equipment.

These braces are rigid, and thus cannot be bent by forces applied to the electrical lines. But the electrical lines may be subjected to unusually heavy loads due to frost, snow, or wind.

Given that these loads do not lead to any deformation of the equipment, the above-mentioned unusually heavy loads may cause the line to break, which in turn would cause torque that could lead the pole to break.

To avoid such problems it has been proposed that the equipment be made of a flexible material of glass fiber-reinforced synthetic resin and having a cross section that decreases regularly from the pole.

Ideally this equipment should have the greatest possible longitudinal flexibility, while also being able to support the greatest possible vertical loads. In practice, such a compromise is difficult to realize.

The object of this invention is to create equipment that makes it possible to attain the above-mentioned objective, while also being inexpensive.

### SUMMARY OF THE INVENTION

The equipment of this invention comprises a flexible arm which is provided at one end with means for attaching it to the pole, and at the other end with means for attaching to it an electric line approximately perpendicular to the arm. The arm has a rectangular cross section, with a height of the section being measured in a plane perpendicular to the electrical line and a width being measured in a direction parallel to the electrical line. The height is greater than the width.

According to the invention, the width of this cross section decreases regularly from the point at which the equipment is attached to the post to the point at which it is attached to the electrical line; whereas the height of the cross section is constant; the arm, in the direction of its thickness, has a series of layers of continuous mineral fibers extending in the direction of the arm's length, each separated by a layer of short randomly-oriented short mineral fibers, these fibers and layers being bonded by a synthetic resin.

This succession of layers of mineral fibers coated in a synthetic resin gives the equipment, by virtue of its geometry, great longitudinal flexibility, as well as great resistance to vertical loads.

The layers containing continuous fibers extending along the length of the equipment, and embedded in the synthetic resin, because they are disposed in vertical planes, make the equipment extremely resistant to vertical loads, as well as resistant to breaking under high

flexure. Moreover, because the cross section of the equipment has a much greater vertical dimension than in the longitudinal direction of the electric line, and because this section decreases regularly from the pole, the equipment has great longitudinal flexibility.

The layer containing randomly-oriented short fibers makes it possible to distribute the thermal and mechanical stress among the above-mentioned layers of continuous fibers.

Moreover, this intermediate layer of randomly-oriented short fibers makes it possible to perforate the arm. In fact, if the equipment had only the continuous longitudinal fibers, perforation of the equipment would cause delamination.

To increase the equipment's resistance to torsional stress, a layer of a fabric of mineral fibers is placed on each side of the arm between the first layer of short fibers and the next layer of continuous fibers. This fabric should enclose fiber filaments placed at +45° and -45° to the direction of the length of the equipment, which will make it possible to obtain optimal resistance to torsion.

Thus, the functions of the different successive layers of the equipment, according to the invention, jointly contribute to making a device that has the desired mechanical properties.

According to a preferred embodiment, the proportion of continuous fibers is greater than that of short fibers.

This proportion is based on the primary role of the continuous fibers in obtaining the sought-after mechanical properties. It is also advisable to use the greatest possible number of continuous fibers.

According to a preferred version of the invention, certain layers of short fibers are separated from the next layer of continuous fibers by supplementary layers of short fibers that extend over only a part of the length of the arm from the end that attaches to the post. The lengths of these layers of short fibers diminish progressively from the exterior to the middle of the thickness of the arm to produce a regularly decreasing thickness of the arm from the post to the end of the equipment intended to support the electric line.

Preferably, the exterior surface of the arm is covered by a plastic coating resistant to electric arcing, inclement weather, and ultra-violet rays, made of a material such as an ethylene-propylene-diene-methylenic (EPDM) copolymer.

According to another aspect of the invention, the procedure for manufacturing insulating equipment for electric line poles comprises the following steps:

making strips containing a layer of continuous fibers that extend along the length of the strip and a layer of randomly-oriented short fibers pre-impregnated with polyester resin and possibly strips of a fabric of fibers at ±45° to the lengthwise direction of the strip;

cutting these strips to the dimensions of the desired length and height of the equipment;

stacking the different strips according to the desired placement;

preheating this stack to a temperature below the polymerization temperature of the polyester resin;

placing the stack in a mold, and heating and applying pressure to mold the stack.

Other features and advantages of the invention will be described below.

The following drawings are given as nonlimiting examples:

#### BRIEF DESCRIPTION OF THE DRAWINGS

FIG. 1 is an elevation view showing the upper part of a pole outfitted with the equipment described by this invention;

FIG. 2 is a top plan view of FIG. 1;

FIG. 3 is an elevation view in transverse cross section, at a larger scale, of the equipment;

FIG. 4 is a schematic elevation view of part of a layer containing continuous longitudinal fibers;

FIG. 5 is a schematic elevation view of part of a layer containing randomly-oriented continuous fibers;

FIG. 6 is a schematic elevation view of part of a fabric of fiber filaments disposed at  $\pm 45^\circ$ ;

FIG. 7 is a schematic plan view in longitudinal cross section showing the juxtaposition of the layers of FIGS. 4, 5 and 6;

FIG. 8 is a schematic plan view of the equipment in longitudinal cross section showing the different layers of this equipment according to the invention;

FIG. 9 is a longitudinal cross-section of a mold illustrating the procedure for manufacturing the equipment according to the invention.

#### DETAILED DESCRIPTION OF THE PREFERRED EMBODIMENTS

In the embodiment of FIGS. 1 and 2 a lateral equipment 100 is constituted by a flexible arm 1 having at one end a support 2 to attach it to a pole 3 and at its other end a tip 4 carrying a cable clamp to which is attached an electric line 6 extending perpendicularly to arm 1. Arm 1 has a rectangular transverse cross section (see FIG. 3). The height 1 of this section measured in a plane perpendicular to the electrical line 6 is clearly greater than the width e of this section measured in a direction parallel to the electrical line 6 in the plane of FIG. 2.

As can be observed in FIG. 2, the width e of the transverse cross section of arm 1 decreases regularly from the support 2 of the attachment to the pole 3, toward the tip 4 for attachment to the electrical line 6. In addition, the height 1 of this section is constant (see FIG. 1).

The arm 1 has in the direction of its thickness e, i.e., 45 in the plane of FIG. 2, a series of layers 7a, 7b, 7c, 7d of continuous glass fibers 10 (see FIGS. 4, 7, 8) extending in the direction of the length L of arm 1. These layers 7a, 7b, 7c, 7d are separated by layers 8a, 8b, 8c, 8d of randomly-oriented short glass fibers 11 (see FIGS. 5, 7, 50 8). These two layers and their fibers are bonded by a synthetic resin, such as a polyester resin.

In addition, layers 9a, 9b of glass fiber fabric are disposed (see FIG. 8), one on each side of the arm 1, between the first layer of short fibers 11 and the next 55 layer 7b of continuous fibers 10.

The different layers are distributed symmetrically on either side of the neutral fiber N of arm 1.

The different layers, such as 7a, 8a, 9a are bonded by polymerization of the synthetic resin, using a pressure 60 molding operation that will be described below.

The proportion of continuous fibers 10 preferably should be greater than that of short fibers 11. The continuous fibers 10 should account for approximately 80% of the weight of all the fibers, the short fibers 11 thus accounting for approximately 20% of the total.

The continuous fibers 10 and short fibers 11 preferably should account for 50 to 60% of the total mass, the

proportion of synthetic resin thus accounting for 40 to 50%.

The fabric 9a (or 9b) (see FIG. 6) has a first series of filaments 12a of parallel glass fibers placed at  $+45^\circ$  with respect to the direction of the length L of the arm 1, and a second series of filaments 12b of parallel fibers placed at  $-45^\circ$  with respect to that direction.

Furthermore, one can observe in FIG. 8 that certain layers of short fibers such as 13a, 13b, 13c extend along only a part of the length L of the arm 1 from the support 2 where it is attached to the pole 3. The lengths of these layers of short fibers 13a, 13b, 13c diminish progressively from the exterior toward the middle N of the thickness of the arm 1 to produce a thickness e that decreases regularly, as indicated in FIG. 2.

Moreover, the exterior surface of the arm 1 is covered (see FIG. 3) with a coating 14 made of elastomer resistant to electric arcing, inclement weather, and ultra-violet rays, such as an ethylene-propylene-diene-methylenic (EPDM) copolymer.

The support 2 that attaches the arm 1 to the pole 3, as well as the tip at end 4, preferably are made of aluminum and are fixed to the arm 1 by gluing. Of the common metals, aluminum has the expansion coefficient closest to that of the composite material (glass fibers, polyester resin) of which arm 1 is made, so that the bonding of the support 2 and the tip 4 to the arm 1 do not run the risk of being affected by variations in temperature.

Following is a detailed description of the procedure for manufacturing the equipment in accordance with the invention.

In a first step, a strip is made that comprises, in succession, a layer of continuous glass fibers 10 that extend along the length of the strip, a layer of randomly-oriented short fibers 11, and a layer of fabric 9a of glass fiber filaments 12a, 12b forming an angle of  $\pm 45^\circ$  with respect to the length L of the strip. Together these layers are pre-impregnated with a polyester resin.

The make-up of this strip might be, for example, as follows:

polyester resin: 18%  
shrink-proof thermoplastic agent: 12%  
adjuvant, coloring catalyst: 3%  
mineral fillers: 12%  
glass fibers: 55%

The strips, pre-impregnated with polyester resin, are then cut to the dimensions of the arm 1.

The strips are then stacked following the distribution illustration in FIG. 8.

The stack thus made is then placed in a high-frequency pre-heater for heating to approximately 70° C. (a temperature less than the polymerization temperature of the polyester resin).

This preheating makes it possible to significantly diminish the thermal stress within the material when the molding is performed.

The resulting stack 15 is then placed in a mold (see FIG. 9) of two parts 16 and 17 placed in a press. The stack 15 is heated to the polymerization temperature of the polyester resin, all the while applying pressure (see arrows F in FIG. 9).

The stack 15 is then withdrawn from the mold, trimmed, cooled, and then sanded or pumiced to obtain the best possible surface.

The aluminum support 2 and tip 4 are then bonded to the ends of the stack.

The adhesive used for this can be a semi-conductive adhesive to avoid problems of partial discharges. The exterior surface of the arm thus obtained is then coated with a primary adhesive and then a coating of EPDM.

For a given flexibility, the equipment thus produced 5 is more resistant to vertical loads than equipment of constant cross section and inertia produced, for example, by drawing through a die.

Thus, such equipment produced in accordance with the invention, with a length L equal to 150 cm, a height 10 1 equal to 90 mm, and a thickness e decreasing from 25 to 20 mm supports a static vertical load greater than 240 daN and has a longitudinal flexibility greater than 5 mm/daN.

These mechanical properties result from the fact that 15 the equipment encompasses a large proportion of continuous longitudinal fibers 10. The fabric having glass fiber filaments 12a and 12b forming angles of +45° and -45° with the direction of the length L of the equipment makes it possible to increase the torsion resistance 20 of the equipment, while the layers enclosing the randomly-oriented short glass fibers 11 make it possible to distribute the thermal and mechanical stresses among the fabric and the adjacent long-fiber layers and to 25 perforate the arm 1 without risk of delamination. 25

In the case in which the equipment is intended to withstand less torsional stress, the presence of fabric 9a, 9b is not necessary.

It should be understood that the invention is not limited to the embodiments which have just been described; various modifications can be made within the framework of the invention. 30

Moreover, the glass fibers can be replaced by other mineral fibers such as rock fibers.

Also, the polyester resin can be replaced by a heat set 35 or thermoplastic resin.

In addition, the dimensions of the arm 1 can be modified according to needs.

Also, arm 1, instead of being perpendicular to the pole 3 can be placed at an oblique angle. 40

In addition, in the process for manufacturing the equipment, instead of stacking the strips of pre-impregnated fibers, cut to the dimensions L and 1 of the equipment, on top of one another, one can proceed as follows:

A sheet having a length L of the equipment and having a layer of continuous fibers and a layer of short fibers pre-impregnated with resin as wound so as to form a flattened spiral comprising strips of maximum width equal to 1 bonded to one another. Thus, a stack is 50 made composed of successive layers of continuous fibers and short fibers.

To obtain a decreasing thickness, variable length strips, such as the short-fiber layers (13a, 13b, 13c) shown in FIG. 8, are intercalated between the layers of 55 the spiral.

I claim:

1. A method for making an elongated insulating support arm having a preselected length dimension, a pre-selected constant width dimension, and a preselected maximum thickness dimension substantially less than the width dimension, for cantilevered mounted on an 60

electric pole to support an electric line extending substantially parallel to the thickness dimension of the arm, the method comprising the steps of:

providing an at least two-ply sheet having a first dimension equal to the desired length of the support arm and a second dimension perpendicular to the first dimension, the sheet being composed of a first ply of continuous fibers extending parallel to the first dimension and a second ply of randomly-oriented short fibers impregnated with a polymerizable resin;

winding the sheet onto itself parallel to the first dimension to form a flattened roll having length, width, and thickness dimensions approximately equal to the respective preselected length, width, and thickness dimensions of the support arm;

preheating the wound roll to a temperature lower than the polymerization temperature of the impregnating resin; and

curing the preheated wound roll in a mold under pressure at a temperature above the polymerization temperature of the resin to obtain an elongated composite fiber-reinforced support arm having length, width, and thickness dimensions equal to said respective preselected length, width, and thickness dimensions, with a first end of the arm being adapted for cantilevered mounting on an electric pole with the width dimension of the arm vertical and a second end being adapted to support an electric line extending substantially parallel to the thickness dimension of the arm, the thickness dimension being made up of successive layers of the two-ply sheet bonded together by the cured resin, with the continuous fibers of the first plies extending parallel to the length dimension of the arm.

2. The method of claim 1 wherein the step of winding the sheet onto itself to form a flattened wound roll comprises intercalating, between the wound layers, strips consisting of sheets selected from continuous fiber layers and short fiber layers, each strip having a width dimension about the same as the preselected width dimension of the support arm and a length dimension less than the preselected length dimension of the arm, the length dimensions of successive strips being different so as to produce a decreasing thickness of the molded support arm in the direction from the first end to the second end. 45

3. The method of claim 1 wherein the preheating step comprises applying a high frequency electromagnetic field to raise the temperature of the wound roll to about 70° C.

4. The method of claim 1 wherein the step of providing an at least two-ply sheet comprises providing a three-ply sheet, with a third ply composed of a fabric having a first series of parallel filaments disposed at an angle of about 45° with respect to the first dimension of the sheet and a second series of parallel filaments disposed at an angle of approximately 90° with respect to the first series.

\* \* \* \* \*

UNITED STATES PATENT AND TRADEMARK OFFICE  
CERTIFICATE OF CORRECTION

PATENT NO. : 5,009,734

DATED : 23 April 1991

INVENTOR(S) : Michel THEROND

It is certified that error appears in the above-identified patent and that said Letters Patent is hereby corrected as shown below:

Col. 3, line 35: "l" should be --l--.  
Col. 3, line 37: "e" should be --e--.  
Col. 3, line 39: "e" should be --e--.  
Col. 3, line 43: "l" should be --l--.  
Col. 3, line 45: "e" should be --e--.  
Col. 4, line 14: "e" should be --e--.  
Col. 5, line 11: "l" should be --l--.  
Col. 5, line 11: "e" should be --e--.  
Col. 5, line 43: "l" should be --l--.  
  
Col. 5, line 50: "l" should be --l--.

Signed and Sealed this  
Fifth Day of January, 1993

*Attest:*

DOUGLAS B. COMER

*Attesting Officer*

*Acting Commissioner of Patents and Trademarks*